

## UNITED STATES PATENT OFFICE

2,066,842

## COATING MAGNESIUM

Herman J. Lodeesen, Detroit, Mich., assignor, by  
mesne assignments, to The Patents Corpora-  
tion, Detroit, Mich., a corporation of Michigan

No Drawing. Application December 22, 1934,  
Serial No. 758,825

1 Claim. (Cl. 148—6)

This invention relates to coating magnesium to increase its resistance to corrosion and to form a base for paint, lacquer or the like.

It has been known for some time that a dilute 5 solution of acid phosphates can be employed for producing on the surface of magnesium and magnesium alloys a coating which increases the resistance of the metal to corrosion and forms a good base for paint. It has been discovered that 10 a better coating for these purposes can be formed by the use of oxalic acid, and this invention relates to the proper use of oxalic acid for producing the best results.

A coating on magnesium can be formed by employing a solution of oxalic acid at various 15 temperatures and containing various materials in addition to the oxalic acid. Also magnesium can be coated by a number of other organic acids, but so far as found, the best coating can be produced by a somewhat dilute solution consisting 20 essentially of oxalic acid and employed at approximately boiling temperature.

A 1% solution of oxalic acid at boiling temperature saturated with magnesium produces a very 25 satisfactory coating on magnesium and magnesium alloys in from two to ten minutes, depending upon the nature of the surface and the alloy. The saturation of the solution may be obtained merely by boiling magnesium articles therein, if 30 desired, in which case the first articles are pickled for a considerable length of time and the final coatings on these first articles are not as good as subsequent coatings. It is preferable to supply a compound of magnesium or some other compound 35 for starting purposes. A small amount of magnesium carbonate, such as  $\frac{1}{2}$  gram to 100 cc. water is sufficient to form a good coating solution, or an equivalent amount of magnesium oxide may be used, or other magnesium compound. 40

It has been found also that in employing a 45 fresh solution, a small amount of a compound containing substantially any metal below magnesium in the electromotive series will take the place of the magnesium compound for effecting a prompt coating action. Among the compounds which have been employed effectively for this 50 purpose are compounds of iron, zinc, cadmium, cobalt, copper, silver, molybdenum, manganese and aluminum. As little as one-tenth per cent of aluminum sulphate is generally effective for making the solution coat promptly. After the solution has been used to coat a few panels, the work is satisfactory regardless of whether or not 55 any compound of any metal has been added and

where a compound such as aluminum sulphate, or any other compound of the metals mentioned is employed for purposes of obtaining a coating when starting a new solution, there is no need of adding any more of this compound when 5 replenishing the solution, since as satisfactory a coating for most purposes is obtained without any such addition.

There are a number of the metals mentioned 10 which change the appearance of the coating to a certain extent, manganese dioxide, iron compounds and compounds of molybdenum and copper when employed in small amounts, producing a darker coating, and the manganese and iron in particular seem to affect the crystallization. Normally the coating is exceedingly fine grained and 15 for most purposes this is preferable. With the use of iron under some conditions the crystals become so coarse as to resemble what is known in the trade as sparkle, in connection with the phosphate coatings, but this may be avoided by using 20 small amounts of the iron and at proper temperatures.

As previously indicated, coatings may be obtained at lower temperatures, and even at room 25 temperature a coating furnishing some advantages may be obtained, particularly with the use of some compounds other than magnesium, the use of ferric salts being particularly good for this purpose. However these coatings are not as 30 satisfactory as the coating resulting from the use of oxalic acid at approximately boiling temperatures, which produces a thin fine grained coating so adherent that it is a substantially integral portion of the coated article and does not flake off 35 when the article is bent. It greatly increases the resistance of the article to corrosion and forms a particularly good base for paint. It has been found by tests to form a materially better base 40 for paint than the phosphate coatings which have been produced hitherto.

While all the dicarboxylic and hydroxydicarboxylic acids of the fatty acid series and the carboxylic acids having but one carboxyl group and the sulphonic acids of the aromatic series and 45 even some additional acids, such as glycolic and citric of the fatty acid series and some other acids of the aromatic series, have a coating effect upon magnesium when properly employed, none of these is as satisfactory as the coating produced by 50 oxalic acid employed in the manner mentioned above. The nearest equivalents of oxalic acid are, as should be expected, those most closely related thereto, that is, the other dicarboxylic acids of the fatty acid series. Succinic, glutaric and adipic 55

acids have been used with good results and might be employed if oxalic acid were not available, but these other acids are higher in price than oxalic acid and are somewhat inferior in results.

- 5 While coatings may be produced by weaker solutions, and stronger solutions than 1% oxalic acid, the weaker solutions require a longer time and the stronger solutions have a tendency to pickle the work to a greater extent than the 1% solution, and, therefore, approximately 1% solution is the preferable concentration. This forms,

on a surface the major ingredient in which is magnesium, a substantially integral, thin, adherent coating of magnesium oxalate.

What I claim is:—

A method of coating a surface the major ingredient of which is magnesium, which consists in treating said surface with an approximately 1% solution of oxalic acid at approximately boiling temperature.

HERMAN J. LODEESSEN. 10